

# UNITED STATES PATENT OFFICE.

ADÉLE ELISE PIRSCH-BAUDVIN, OF PARIS, FRANCE.

## IMPROVEMENT IN ALLOYS TO RESEMBLE SILVER.

Specification forming part of Letters Patent No. 142,760, dated September 16, 1873; application filed May 29, 1873.

*To all whom it may concern:*

Be it known that I, ADÉLE ELISE PIRSCH-BAUDVIN, of Paris, in the Republic of France, have invented certain new or Improved Metallic Alloy Resembling Silver, of which the following is a specification:

The nature of said invention consists in the production of a metallic alloy resembling silver more closely than any alloys heretofore produced in color, specific gravity, malleability, ductility, ring, and general characteristics.

For these purposes the following metals are combined: Copper, nickel, tin, zinc, cobalt, and iron.

The following proportions are suitable, and produce a very white and silver-like metal:

|              |              |
|--------------|--------------|
| Copper ..... | 71.00 parts. |
| Nickel ..... | 16.50 parts. |
| Cobalt ..... | 1.75 parts.  |
| Tin .....    | 2.50 parts.  |
| Iron .....   | 1.25 parts.  |
| Zinc .....   | 7.00 parts.  |
| <hr/>        |              |
|              | 100.00       |

In some cases, also, a small proportion—say, one-half per cent.—of aluminium is added.

The nickel is first alloyed with an equal weight of copper, and the zinc also with copper in the proportion of six parts of the former to ten of the latter. The nickel alloy, the iron,

the remainder of the copper, the cobalt (in the state of black oxide,) and charcoal are then placed together in a plumbago crucible. The charge is covered with charcoal and the whole is exposed to a high heat. When the materials are melted the heat is reduced and the alloy of zinc and copper is added when the heat is such that it will just melt freely. This having been done, the crucible is taken from the fire and stirred with a rod of hazelwood. The tin is then added. It is wrapped in paper and dropped into the crucible. The metal is again stirred and at once cast into ingot-molds. It can afterward be rolled and otherwise worked as silver is worked.

Much of the zinc is volatilized in the process of melting, and the proportion ultimately remaining in the alloy is small.

The superiority of this alloy over other silver-like alloys depends mainly upon the influence of cobalt. If the cobalt be omitted from the alloy it will cease to have a silver-like appearance.

What I claim as my invention is—

The manufacture of an alloy resembling silver, substantially in the manner described.

ADÉLE ELISE PIRSCH-BAUDVIN.

Witnesses:

M. TAUSSUPANSE,  
A. LAFAGSE.